

# UNITED STATES PATENT OFFICE.

CLARENCE ROSCOE KING, OF WORCESTER, MASSACHUSETTS, ASSIGNOR TO NORTON COMPANY, A CORPORATION OF MASSACHUSETTS.

## PROCESS OF MAKING ABRASIVE WHEELS.

1,208,330.

Specification of Letters Patent. Patented Dec. 12, 1916.

No Drawing.

Application filed May 28, 1914. Serial No. 841,678.

*To all whom it may concern:*

Be it known that I, CLARENCE ROSCOE KING, a citizen of the United States, residing at Worcester, in the county of Worcester and State of Massachusetts, have invented a new and useful Process of Making Abrasive Wheels, of which the following is a specification.

This invention relates to a process of making abrasive wheels and more specifically to a process of making abrasive wheels in which a supplemental bond is embodied.

The details of my improved process are fully described in the following specification and the novel features thereof are specifically defined in the appended claim.

My improved process is more particularly applicable to abrasive wheels having a porous unitary structure. Such wheel may be generally defined as having the abrasive material united and held together by some form of silicate binder and are classified commercially as vitrified wheels and silicate wheels. In the first class, the silicate binder is in the

form of clay mixed with other mineral silicates which are partially fused by burning in a kiln, and form a porous mass more or less resembling porcelain or glass, in which the abrasive particles are firmly embedded.

In the so-called "silicate" wheels, the principal binding constituent is silicate of soda, commonly known as "water glass." This silicate, together with certain mineral powders, is mixed with the loose grains of abrasive material.

After being molded to the desired shape and size, the wheel thus formed is dried and is then heated to a sufficient temperature to cause the silicate of soda to react with the other minerals to form a hard, porous mass which securely holds the abrasive grains in place. Each

of these two types of wheels is distinguished by the use of a silicate binder and by the fact that the wheel thus formed possesses a porous, unitary structure. The silicate binder in either type may be considered as a thin envelop inclosing and fixing the abrasive grains in position.

When the wheel is in use the grains upon the periphery thereof are subject to the abrasive action between the wheel and the work and also to severe torsional and impact strains. The silicate binder, when formed into a porous mass having the abrasive grains distributed therethrough, pos-

sesses substantially no resilience and only a very slight degree of toughness. As the qualities of resilience and toughness are most essential for resisting the torsional and impact strains, I have devised the process described in this application for supplementing and reinforcing the silicate binder.

In carrying out this process, I make use of a material which can be incorporated in the voids of the porous structure of the wheel and which can thereafter be given a permanent set by the application of heat, being thus changed into a hard, tough substance which cannot be thereafter liquefied at any temperature which will be attained in grinding operations. I have found that the so-called synthetic resins are particularly adapted for this purpose. These resins are manufactured under various trade names such as bakelite, condensite, amberoid, plastic, fenoform, and the like, and they have in common the quality of receiving a permanent set when heated to a moderate temperature.

In practising my improved process, I form an abrasive wheel having a porous unitary structure in the usual manner, and fill the voids of the structure with one of these synthetic resins in solution or in liquid form. The wheel is then heated to a temperature sufficient to give the permanent set to the supplementary bonding material and is then ready for use.

I have found by actual test that wheels thus treated will remove more material per unit of wheel wear and that they act as they would have done if they were originally made several grades harder. They also wear from two to four times longer than similar wheels which do not have the supplemental bond.

I do not wish to be limited to the use of synthetic resins in carrying out my process, as it will be evident that many of the beneficial results of the process may be attained by the use of other materials. It is essential only that they be applied to fill the voids of the grinding wheels, that they can thereafter be given a permanent set, and that having once received this permanent set they cannot again be liquefied at ordinary grinding temperatures. Such materials can be broadly distinguished from the mineral silicates by the term organic.

Although I have described my invention

in connection with abrasive wheels, it will be evident that the same process may be practised in connection with any abrasive instrumentality, whether it is designed for 5 rotation or for use in other ways.

Having thus described my improved process, what I do claim and desire to secure by Letters-Patent is:—

The process of making an abrasive wheel 10 which consists in forming a wheel having a porous structure, dipping said wheel in an unheated solution of synthetic resin, and

therafters heating said wheel and thereby transforming said resin into a hard tough supplemental bonding material incapable of 15 subsequent liquification by heat.

In testimony whereof I have hereunto set my hand, in the presence of two subscribing witnesses.

CLARENCE ROSCOE KING.

Witnesses:

CHAS. T. HAWLEY,  
C. FORREST WESSON.